# EUROPEAN PATENT APPLICATION

(11) **EP 4 130 301 A1**
(43) Date of publication of application: **08.02.2023**
(21) Application number: 21776156.8
(22) Date of filing: 18.03.2021
(51) Int. Cl.: C21D 6/00, C22C 38/00, H01F 41/02, H01F 1/059, B22F 3/00, B22F 3/02, B22F 3/24

(54) **ANISOTROPIC RARE-EARTH SINTERED MAGNET AND METHOD FOR PRODUCING SAME**

(30) Priority: 26.03.2020 JP 2020055762
(71) Applicant: Shin-Etsu Chemical Co., Ltd., Tokyo 100-0005 (JP)
(72) Inventor: NOMURA, Tadao, Echizen-shi, Fukui 915-8515 (JP); OTSUKA, Kazuki, Echizen-shi, Fukui 915-8515 (JP); KAMATA, Masayuki, Echizen-shi, Fukui 915-8515 (JP)
(74) Representative: Vossius & Partner Patentanwälte Rechtsanwälte mbB
(86) International application number: PCT/JP2021/011007
(87) International publication number: WO 2021/193333

(57) **Abstract**

Provided is an anisotropic rare earth sintered magnet represented by the formula (R₁₋ₐZrₐ)ₓ(Fe_{1-b}Co_{b})_{100-x-y}(M¹_{1-c}M²_{c})_{y} (wherein R is at least one element selected from rare earth elements and Sm is essential; M¹ is at least one element selected from the group consisting of V, Cr, Mn, Ni, Cu, Zn, Ga, Al, and Si; M² is at least one element selected from the group consisting of Ti, Nb, Mo, Hf, Ta, and W; x, y, a, b, and c each satisfy 7 ≤ x ≤ 15 at%, 4 ≤ y ≤ 20 at%, 0 ≤ a ≤ 0.2, 0 ≤ b ≤ 0.5, and 0 ≤ c ≤ 0.9). The anisotropic rare earth sintered magnet includes 80% by volume or more of a main phase composed of a compound of a ThMn₁₂ type crystal, the main phase having an average crystal grain size of 1 um or more, and containing an R-rich phase and an R(Fe,Co)₂ phase in a grain boundary portion. Also provided is a method for producing the anisotropic rare earth sintered magnet, including pulverizing an alloy containing a compound phase of a ThMn₁₂ type crystal; compacting the pulverized alloy under application of a magnetic field to form a compact; and then sintering the compact at a temperature of 800°C or higher and 1400°C or lower. According to the present invention, it is possible to provide an anisotropic rare earth sintered magnet having a compound of a ThMn₁₂ type crystal as a main phase and exhibiting good magnetic properties, and a method for producing the same.

## Description

### Technical Field

The present invention relates to an anisotropic rare earth sintered magnet having a compound of a ThMn₁₂ type crystal as a main phase, and to a method for producing the same.

### Background Art

The demand for rare earth magnets, in particular, Nd-Fe-B sintered magnets is expected to increase more and more in the future and the production amount thereof is expected to increase more and more in the background of motorization of automobiles, high performance and power saving of industrial motors, and the like. On the other hand, since there is concern about the risk that the supply and demand balance of rare earth raw materials will be lost in the future, research on rare earth saving in rare earth magnets has been attracting attention in recent years. Among them, compounds having a ThMn₁₂ type crystal structure have a lower content of rare earths than R₂Fe₁₄B compounds and have good magnetic properties, so that they have been actively studied as next-generation magnetic materials.

For example, PTL 1 reports permanent magnets made of alloys containing a hard magnetic phase having a ThMn₁₂ type tetragonal structure and a nonmagnetic phase. Here, it is shown that by adding at least one element selected from Cu, Bi, Mg, Sn, Pb, and In to an intermetallic compound mainly composed of a rare earth element-Fe, a phase having a melting point lower than that of the main phase and being nonmagnetic is precipitated.

In addition, PTL 2 reports a rare earth permanent magnet having a main phase and a grain boundary phase, wherein the main phase is an R-T compound having a ThMn₁₂ type crystal structure (wherein R is one or more rare earth elements in which La is essential, and T is Fe, or Fe and Co, or an element in which a part thereof is substituted with M (one or more elements selected from Ti, V, Cr, Mo, W, Zr, Hf, Nb, Ta, Al, Si, Cu, Zn, Ga, and Ge)), wherein the grain boundary phase has a cubic crystal structure, and has 20% or more of a La-rich phase σ having a La composition ratio of 20 at% or more in cross-sectional area ratio. By including the non-magnetic cubic La-rich phase in the grain boundary portion, a magnetic separation effect between the main phases and an interfacial distortion reduction effect between the grain boundary phase and the main phase are obtained.

PTL 3 reports rare earth magnets including a main phase having a ThMn₁₂ type crystal structure and a subphase containing any one of a Sm₅Fe₁₇ base phase, a SmCos base phase, a Sm₂O₃ base phase, and a Sm₇Cu₃ base phase, wherein the subphase has a volume fraction of 2.3 to 9.5%. Among these subphases, the Sm₅Fe₁₇ base phase and the SmCo₅ base phase are magnetic phases exhibiting magnetic anisotropies higher than that of the main phase, and isolate crystal grains of the main phase from each other and prevent a domain wall in the main phase from moving, thereby improving the magnetization and coercive force of the magnets. On the other hand, the Sm₂O₃ base phase and the Sm₇Cu₃ base phase are non-magnetic phases, and by isolating the crystal grains of the main phase from each other, the magnetization reversal of the main phase is prevented from propagating to the surroundings, thereby improving the magnetization and coercive force of the magnets. PTL 3 also describes that the Sm₇Cu₃ base phase is a non-equilibrium phase.

PTL 4 reports alloys for rare earth magnets which have a main phase and one or more subphases and whose composition satisfies R(Fe,Co)_{w-z}Ti_{z}Cu_{α} (wherein R is at least one of rare earth elements, 8 ≤ w ≤ 13, 0.42 ≤ z < 0.70, and 0.40 ≤ α ≤ 0.70). In addition, PTL4 also describes that the subphase is mainly a crystal phase in which 50 mol% or more of the entire subphase has a Cu composition, and the crystal structure of the subphase is a KHg₂ type.

PTL 5 reports rare earth permanent magnets having a structure RₓFe_{100-x-y}(V₁₋ₐSiₐ)_{y} (wherein R represents one or more rare earth elements including Y, x = 5.5 to 18 at%, y = 8 to 20 at%, and a = 0.05 to 0.7) and having a ThMn₁₂ type body-centered tetragonal structure as a main phase. It is described that this composition alloy is composed of a main phase and a rare earth-rich phase and does not contain an RFe₂ phase.

### Citation List

### Patent Literature

PTL 1: JP 2001-189206 A
PTL 2: WO 2017/164312 A
PTL 3: JP 2017-112300 A
PTL 4: JP 2019-044259 A
PTL 5: JP 06-231920 A

### Summary of Invention

### Technical Problem

As described above, in order to obtain good magnetic properties in magnets having a ThMn₁₂ type compound as a main phase, it has been proposed to form a structure composed of a main phase and a grain boundary phase as in Nd-Fe-B base magnets, and non-magnetic phases such as a La-rich phase (PTL 2) and an R-Cu phase (PTLs 1 and 4) have been studied as a grain boundary phase. However, in practice, these phases are segregated at grain boundary triple junctions or the like and it is difficult to form an intergranular grain boundary phase, and there is a problem in that it is difficult to obtain a structure in which the surface of the main phase grains is covered with the grain boundary phase.

Further, in PTL 3, the surfaces of the main phase grains are surrounded by a Sm₅Fe₁₇ base phase or a SmCos base phase, which is a magnetic phase exhibiting high magnetic anisotropy, and the coercive force is improved by pinning the domain wall by this phase. However, since it is difficult for the Sm₅Fe₁₇ base phase and the SmCo₅ base phase to be in phase equilibrium with the ThMn₁₂ type compound, it is difficult to realize a structural form in which the surfaces of the crystal grains of the main phase are surrounded by these phases.

On the other hand, PTL 5 proposes alloys composed of a ThMn₁₂ main phase and an R-rich phase. However, since the composition range in which only two phases are formed in the R-Fe-V-Si quaternary system is extremely limited, it is difficult to produce this structure with good reproducibility.

The present invention has been made in view of the above problems, and an object of the present invention is to provide an anisotropic rare earth sintered magnet having a compound of a ThMn₁₂ type crystal having good magnetic properties as a main phase.

### Solution to Problem

As a result of intensive studies to achieve the above object, the present inventors have found that high coercive force is exhibited when an R-rich phase and an R(Fe,Co)₂ phase are present in a grain boundary portion in anisotropic rare earth sintered magnets having a compound of a ThMn₁₂ type crystal as a main phase, and completed the present invention.

Accordingly, the present invention provides the following anisotropic rare earth sintered magnet and a method for producing the same.
(1) An anisotropic rare earth sintered magnet represented by the formula (R₁₋ₐZrₐ)ₓ(Fe_{1-b}Co_{b})_{100-x-y}(M¹_{1-c}M²_{c})_{y} (wherein R is at least one element selected from rare earth elements and Sm is essential; M¹ is at least one element selected from the group consisting of V, Cr, Mn, Ni, Cu, Zn, Ga, Al, and Si; M² is at least one element selected from the group consisting of Ti, Nb, Mo, Hf, Ta, and W; x, y, a, b, and c each satisfy 7 ≤ x ≤ 15 at%, 4 ≤ y ≤ 20 at%, 0 ≤ a ≤ 0.2, 0 ≤ b ≤ 0.5, and 0 ≤ c ≤ 0.9), the magnet including 80% by volume or more of a main phase composed of a compound of a ThMn₁₂ type crystal, the main phase having an average crystal grain size of 1 pm or more, and containing an R-rich phase and an R(Fe,Co)₂ phase in a grain boundary portion.
(2) The anisotropic rare earth sintered magnet as set forth in (1), wherein the R-rich phase and the R(Fe,Co)₂ phase are contained in an amount of 1% by volume or more in total.
(3) The anisotropic rare earth sintered magnet as set forth in (1) or (2), wherein the R-rich phase contains R in an amount of 40 at% or more.
(4) The anisotropic rare earth sintered magnet as set forth in any one of (1) to (3), wherein the R(Fe,Co)₂ phase is a phase exhibiting ferromagnetism or ferrimagnetism at room temperature or higher.
(5) The anisotropic rare earth sintered magnet as set forth in any one of (1) to (4), wherein a Sm/R ratio in an inner portion of the main phase grain is lower than Sm/R ratios of the R-rich phase and the R(Fe,Co)₂ phase.
(6) The anisotropic rare earth sintered magnet as set forth in any one of (1) to (5), wherein a Sm/R ratio in an inner portion of the main phase grain is lower than a Sm/R ratio in an outer shell portion of the main phase grain.
(7) The anisotropic rare earth sintered magnet as set forth in (5) or (6), wherein Sm is not contained in an inner portion of the main phase grain.
(8) The anisotropic rare earth sintered magnet as set forth in any one of (1) to (7), wherein the magnet exhibits a coercive force of 5 kOe or more at room temperature, and a temperature coefficient β of the coercive force is -0.5%/K or more.
(9) A method for producing the anisotropic rare earth sintered magnet as set forth in any one of (1) to (8), including: pulverizing an alloy containing a compound phase of a ThMn₁₂ type crystal; compacting the pulverized alloy under application of a magnetic field to form a compact; and then sintering the compact at a temperature of 800°C or higher and 1400°C or lower.
(10) The method for producing an anisotropic rare earth sintered magnet as set forth in (9), including: pulverizing and mixing an alloy containing a compound phase of a ThMn₁₂ type crystal and an alloy having a higher R composition ratio and a higher Sm/R ratio; and compacting the mixture under application of a magnetic field to form a compact.
(11) The method for producing an anisotropic rare earth sintered magnet as set forth in (9) or (10), including: bringing a material containing Sm into contact with a sintered body having a compound phase of a ThMn₁₂ type crystal as a main phase; and subjecting to heat treatment at a temperature of 600°C or higher and a sintering temperature or lower to diffuse Sm into the sintered body.
(12) The method for producing an anisotropic rare earth sintered magnet as set forth in (11), wherein the material containing Sm to be brought into contact with the sintered body is at least one selected from Sm metal, Sm-containing alloy, Sm-containing compound, and Sm-containing vapor, and a form thereof is at least one selected from powder, thin film, thin strip, foil, and gas.
(13) The method for producing an anisotropic rare earth sintered magnet as set forth in any one of (9) to (12), including subjecting the sintered body to heat treatment at a temperature of 300 to 900°C.

### Advantageous Effects of Invention

According to the present invention, it is possible to obtain anisotropic rare earth sintered magnets having a compound of a ThMn₁₂ type crystal as a main phase and exhibiting good magnetic properties.

### Description of Embodiments

Hereinafter, embodiments of the present invention will be described. A magnet according to the present invention is an anisotropic rare earth sintered magnet which is represented by the following formula (R₁₋ₐZrₐ)ₓ(Fe_{1-b}Co_{b})_{100-x-y}(M¹_{1-c}M²_{c})_{y}, has a compound of a ThMn₁₂ type crystal as a main phase, contains 80% by volume or more of a main phase composed of the compound of a ThMn₁₂ type crystal, has an average crystal grain size of the main phase of 1 pm or more, and contains an R-rich phase and an R(Fe,Co)₂ phase in a grain boundary portion. First, each component will be described below. Here, x, y, a, b, and c satisfy 7 ≤ x ≤ 15 at%, 4 ≤ y ≤ 20 at%, 0 ≤ a ≤ 0.2, 0 ≤ b ≤ 0.5, and 0 ≤ c ≤ 0.9, respectively.

The R-rich phase is a phase having a higher concentration of rare earth elements than the main phase. The R(Fe,Co)₂ phase has a MgCu₂ structure and is a compound phase called a Laves phase. As described above, since the composition range is wide, the anisotropic rare earth sintered magnet of the present invention can be easily produced with good reproducibility.

R is one or more elements selected from rare earth elements, and Sm is essential. Specifically, R essentially contains Sm, and may be a combination of Sm and one or more elements selected from Sc, Y, La, Ce, Pr, Nd, Eu, Gd, Tb, Dy, Ho, Er, Tm, Yb, and Lu. R is an element necessary for forming a compound having a ThMn₁₂ type crystal structure as a main phase. The content of R is 7 at% or more and 15 at% or less. The content is more preferably 8 at% or more and 12 at% or less. When the content is less than 7 at%, an α-Fe phase is precipitated and it is difficult to sinter, and on the other hand, when the content exceeds 15 at%, the volumetric ratio of the ThMn₁₂ type compound phase is lowered and good magnetic properties cannot be obtained. Since the ThMn₁₂ type compound exhibits a particularly high anisotropic magnetic field H_{A} when R is Sm, Sm is essential for the anisotropic rare earth sintered magnet of the present invention. When there is no difference in Sm concentration between the inner portion and the outer shell portion of the main phase grain, Sm contained in R is preferably 5% or more, more preferably 10% or more, and particularly preferably 20% or more of R in terms of atomic ratio. When the Sm ratio is in such a range, the effect of increasing H_{A} is sufficient, and a high coercive force can be obtained.

On the other hand, since Sm is less produced than Y, La, Ce, Pr, Nd and the like and has a restriction in terms of resources, it is preferable to utilize Sm as effectively as possible. Therefore, as a structural form in which Sm is concentrated in the outer shell portion of the main phase grain, a high coercive force may be obtained with a smaller Sm content. In the case of having a structure in which the Sm concentration is different between the inner portion and the outer shell portion of the main phase grain as described above, the amount of Sm contained in R is preferably 0.1 at% or more and 50 at% or less of R in terms of atomic ratio. It is more preferably 0.2 at% or more and 40 at% or less, and particularly preferably 0.5 at% or more and 30 at% or less. More preferably, R is a combination of Sm and one or more elements selected from Y, La, Ce, Pr, and Nd.

Zr substitutes for R in the ThMn₁₂ type compound and has an effect of enhancing the phase-stability. The content of Zr substituting for R is 20% or less of R in atomic ratio. If it exceeds 20%, H_{A} of the ThMn₁₂ type compound is decreased and it is difficult to obtain a high coercive force.

It is known that a third element M is required together with R and Fe as constituent elements in order to stably exist the ThMn₁₂ type crystal structure. In the anisotropic rare earth sintered magnet of the present invention, M¹ is at least one element selected from the group consisting of V, Cr, Mn, Ni, Cu, Zn, Ga, Al, and Si, and serves as the third element. M¹ is an element which is more likely to form a compound with R than Fe or is less likely to bond with both Fe and R, as compared with M² which also acts as the third element as described later. One of the features of the anisotropic rare earth sintered magnet of the present invention is that the R-rich phase and the R(Fe,Co)₂ phase are present in the grain boundary portion together with the ThMn₁₂ type compound as the main phase in the magnet structure, and by selecting the M¹ element as the third element, it becomes easy to obtain a structure in which these three phases stably coexist. When M¹ and M² are collectively expressed as M, the content of M¹ accounts for at least 10% or more of M in atomic ratio. It is more preferably 30% or more, and still more preferably 50% or more. When the content of M¹ is less than 10%, the R-rich phase among the three phases is not stably formed. In addition, the content of M, which is the sum of M¹ and M², is 4 at% or more and 20 at% or less. When the content of M is less than 4 at%, the main phase of the ThMn₁₂ type compound is not sufficiently formed, and when it exceeds 20 at%, the amount of different phases formed increases and good magnetic properties are not exhibited.

M² is one or more elements selected from Ti, Nb, Mo, Hf, Ta, and W. M² also has an effect of stabilizing the ThMn₁₂ type crystal structure, but when it is excessively contained, carbide such as a M²C phase and a (Fe,Co)₂M² phase which is a MgZn₂ type compound precipitate in the main phase and at the grain boundary portion. In particular, the (Fe,Co)₂M² phase may have a Fe-rich composition rather than a stoichiometric composition, for example, like the Fe₂Ti phase, and may exhibit ferromagnetism, which adversely affects the magnetic properties of the sintered magnet. When only M² is selected as the third element without containing M¹, it is difficult to stably form the R-rich phase. Therefore, in the case of a composition containing M², its content is at least 90% or less of M in atomic ratio.

The anisotropic rare earth sintered magnet of the present invention contains Fe as an essential constituent element together with R and M¹. Further, a part of Fe may be substituted with Co. The substitution with Co has the effect of raising the Curie temperature T_{c} of the ThMn₁₂ type compound as the main phase and increasing the saturation magnetization Ms. The substitution ratio of Co is 50% or less in atomic ratio. When the substitution ratio exceeds 50%, Ms is decreased. The proportion of Fe and Co is the balance of R, Zr, M¹, and M². However, in addition thereto, inevitable impurities taken in from raw materials or mixed in a production process, specifically, H, B, C, N, O, F, P, S, Mg, Cl, Ca, and the like may be contained in an amount of up to 3% by weight in total.

Next, the phases constituting the anisotropic rare earth sintered magnet of the present invention will be described.

The main phase in the anisotropic rare earth sintered magnet of the present invention is composed of an R(Fe,Co,M)₁₂ compound having a ThMn₁₂ type crystal structure. It is preferable that elements such as C, N, and O which are inevitably mixed in a process of producing the sintered magnet are not contained in the main phase. However, when C, N, and O elements are detected by composition analysis using an EPMA (electron probe micro analyzer) due to measurement variation, an adjustment method of an observation sample, influence of detection signals of other elements, and the like, the upper limit of each of them is preferably 1 at% from the viewpoint of obtaining H_{A} of the main phase satisfactorily. The average crystal grain size of the main phase is 1 µm or more, and preferably 1 µm or more and 30 µm or less. The average crystal grain size is more preferably in a range of 1.5 µm or more and 20 pm or less, and particularly preferably 2 pm or more and 10 µm or less. By setting the average crystal grain size in such a range, it is possible to suppress a decrease in residual magnetic flux density Bᵣ due to a decrease in the degree of orientation of crystal grains and a decrease in coercive force H_{cJ}. From the viewpoint of obtaining good Bᵣ and H_{cJ}, the volume fraction of the main phase is 80% by volume or more, preferably 80% by volume or more and less than 99% by volume, and more preferably 90% by volume or more and 95% by volume or less with respect to the entire magnet.

The average crystal grain size of the main phase is a value measured as follows.

After the cross section of the sintered magnet was polished until it becomes a mirror surface, the sintered magnet was immersed in an etching solution (a mixed solution of nitric acid, hydrochloric acid, and glycerin, or the like) to selectively remove the grain boundary phase, and arbitrary 10 or more portions of the cross section were observed with a laser microscope. The cross-sectional area of each grain was calculated from the obtained observation image by image analysis, and the average diameter when these were regarded as circles was taken as the average crystal grain size.

Further, the volume fraction of the main phase is a value measured as follows.

The structure of the anisotropic rare earth sintered magnet was observed and the composition of each phase was analyzed using EPMA to confirm the main phase, the R-rich phase, and the R(Fe,Co)₂ phase. The volume fraction of each phase was calculated as being equal to the area ratio in the backscattered electron image.

In order to effectively utilize Sm, a structure may be adopted in which Sm is concentrated in the outer shell portion of the main phase grains, and grains having a lower Sm concentration in the inner portion of the main phase grains than the outer shell portion are present. In this case, the thickness of the high-Sm outer shell portion is not particularly limited, but is preferably 1 nm to 2 µm, and particularly preferably 2 nm to 1 µm, from the viewpoint of sufficiently obtaining the effect of suppressing nucleation of reverse magnetic domain in the outer shell portion of the main phase grains, and from the viewpoint of suppressing a situation in which the effect of reducing Sm cannot be sufficiently obtained due to an increase in the Sm content in the entire sintered body. Such a form is generated by making the Sm/R ratio (atomic ratio of Sm to R) in the R-rich phase or the R(Fe,Co)₂ phase higher than the Sm/R ratio in the inner portion of the main phase grains. A structure in which Sm is not contained in the inner portion of the main phase grains is more preferable. Further, main phase grains having a uniform Sm concentration distribution may be partially included.

The R-rich phase and the R(Fe,Co)₂ phase are formed in the grain boundary portion of the magnet structure. The grain boundary portion includes grain boundary triple junctions in addition to an intergranular grain boundary phase. Here, the R-rich phase is a phase containing 40 at% or more of R. The present inventors have found that magnets containing three phases, i.e., a main phase, an R(Fe,Co)₂ phase, and an R-rich phase, can be easily obtained when the above-described composition containing the M¹ element is used. For example, in Sm-Fe-Ti ternary system sintered magnets containing no M¹ element, there is a composition region in which three phases of a Sm(Fe,Ti)₁₂ main phase and SmFe₂ and Fe₂Ti (excluding oxides and the like) are in equilibrium, but the Sm(Fe,Ti)₁₂ main phase and the Sm-rich phase are difficult to be in equilibrium at a low temperature of 400°C or lower, and thus the Sm-rich phase is not formed as a stable phase. On the other hand, in the case of Sm-Fe-V ternary system using V which is one of M¹ elements, a Sm-rich phase having a high Sm concentration is formed, and a magnet in which three phases of Sm(Fe,V)₁₂, SmFe₂, and Sm-rich phase are present can be obtained. Further, in Sm-Fe-V-Ti quaternary system containing both M¹ and M², four phases of Sm(Fe,V,Ti)₁₂, Fe₂(V,Ti), SmFe₂, and Sm-rich phase can be stably present. In the anisotropic rare earth sintered magnet of the present invention, based on these findings, a composition containing a predetermined amount of M¹ elements is selected in order to form the R-rich phase and the R(Fe,Co)₂ phase in the grain boundary portion.

The R-rich phase and the R(Fe,Co)₂ phase mainly provide four effects. The first effect is an action of promoting sintering. At the sintering temperature, both the R-rich phase and the R(Fe,Co)₂ phase are melted to form a liquid phase, so that liquid phase sintering proceeds, and sintering is completed more rapidly than solid phase sintering that does not contain these phases. In addition, when the R-rich phase and the R(Fe,Co)₂ phase coexist, the liquid phase formation temperature tends to decrease compared to the case of only one of the phases, and the liquid phase sintering proceeds more rapidly.

The second effect is cleaning of the surface of the main phase grains. Since the anisotropic rare earth sintered magnet of the present invention has a nucleation type coercive force mechanism, it is desirable that the surface of the main phase grains is smooth so that nucleation of reverse magnetic domains is difficult to occur. The R-rich phase and the R(Fe,Co)₂ phase serve to smooth the surfaces of the crystal grains of the ThMn₁₂ type compound in the sintering step or the subsequent aging step, and this cleaning effect suppresses nucleation of reverse magnetic domains, which causes a decrease in coercive force. In particular, the R(Fe,Co)₂ phase has relatively high wettability to the ThMn₁₂ phase compared to other phases having less than 40 at% of R, for example, compound phases such as RM₃, RM₂, R(Fe,Co)M, and R(Fe,Co)₂M₂, and easily covers the surfaces of the main phase grains, and thus has a large cleaning effect.

The third effect is the formation of an intergranular grain boundary phase. In a magnet containing an R-rich phase in the structure, an intergranular grain boundary phase containing a larger amount of R than the main phase is formed between adjacent ThMn₁₂ type compound main phase grains by performing an optimum sintering treatment or aging treatment. As a result, the magnetic interaction between the main phase grains is weakened, and the sintered magnet exhibits a high coercive force. However, since the composition region in which only two phases of the ThMn₁₂ type compound main phase and the R-rich phase are in equilibrium is extremely limited, it is difficult to stably produce such a magnet in consideration of composition variation. A magnet containing three phases of the ThMn₁₂ type compound main phase, the R-rich phase, and the R(Fe,Co)₂ phase can stably form a structure in which the surface of the main phase grain is covered with the intergranular grain boundary phase. In addition, in a magnet in which the R-rich phase does not exist, since it is difficult to form the intergranular grain boundary phase or it is difficult to cover the surface of the main phase grain with the intergranular grain boundary phase, it is difficult to obtain a magnet exhibiting sufficient coercive force.

The fourth effect is to increase the Sm concentration in the grain boundary portion. When the grain boundary diffusion method is applied as a production method in order to obtain a structure in which the Sm concentration is different between the inner portion and the outer shell portion of the main phase grain, the R-rich phase and the R(Fe,Co)₂ phase present in the grain boundary portion become liquid phases during the diffusion treatment, and play a role of diffusing and permeating Sm provided on the sintered body into the inner portion. Therefore, the Sm/R ratio in at least one of the R-rich phase and the R(Fe,Co)₂ phase becomes higher than the Sm/R ratio in the inner portion of the main phase grain. When a dual-alloy method is applied as the production method, the Sm/R ratio in at least one of the R-rich phase and the R(Fe,Co)₂ phase of the sintered body becomes higher than the Sm/R ratio in the inner portion of the main phase grain by using a first alloy mainly composed of the ThMn₁₂ type compound phase and a second alloy having a higher R composition ratio and a higher Sm/R ratio than the first alloy. When Sm is concentrated in the R-rich phase or the R(Fe,Co)₂ phase, the Sm concentration in the outer shell portion of the main phase grain in contact with these grain boundary phases is also increased, and H_{A} is improved to increase the coercive force of the sintered magnet.

As described above, the R-rich phase contains at least 40 at% or more of R. When the content of R is less than 40 at%, the wettability with the main phase is not sufficient, so that the above-described effect is hardly obtained. More preferably, R contains 50 atoms or more, and particularly preferably R contains 60 atoms or more. The R-rich phase may be an R-metal phase such as the above-described Sm phase, or may be an amorphous phase or an intermetallic compound having a high R composition and a low melting temperature, such as R₃(Fe,Co,M), R₂(Fe,Co,M), R₅(Fe,Co,M)₃, and R(Fe,Co,M). In addition, Fe, Co, the M element, and impurity elements such as H, B, C, N, O, F, P, S, Mg, Cl, and Ca may be contained up to 60 at% in total.

On the other hand, the R(Fe,Co)₂ phase is a Laves compound of a MgCu₂ type crystal, but when composition analysis is performed using EPMA or the like, R is contained in an amount of 20 at% or more and less than 40 at% in consideration of measurement variation or the like. Further, a part of Fe and Co may be substituted with the M element. However, the substitution amount of M is within a range in which the MgCu₂ type crystal structure is maintained.

The R(Fe,Co)₂ phase in the anisotropic rare earth sintered magnet of the present invention is a magnetic phase. The term "magnetic phase" as used herein refers to a phase exhibiting ferromagnetism or ferrimagnetism and having a Curie temperature T_{c} of equal to or higher than room temperature (23°C). T_{c} of RFe₂ is equal to or higher than room temperature except for CeFe₂, and T_{c} of CeFe₂ is also equal to or higher than room temperature when 10% or more of R is substituted with another element. On the other hand, with respect to RCo₂ except for GdCo₂, T_{c} of RCo₂ is equal to or lower than room temperature or RCo₂ is a paramagnetic phase, but in the anisotropic rare earth sintered magnet of the present invention, since the substitution atomic ratio of Fe by Co is 0.5 or less, the R(Fe,Co)₂ phase becomes a magnetic phase in most cases. Generally, a soft magnetic phase contained in the structure often adversely affects the magnetic properties, but in the anisotropic rare earth sintered magnet of the present invention, the effect of cleaning the surface of the main phase grains by the R(Fe,Co)₂ phase and the effect of forming the intergranular grain boundary phase are larger, and it is considered that even the magnetic phase contributes to an increase in the coercive force.

The total amount of the R-rich phase and the R(Fe,Co)₂ phase formed is preferably 1% by volume or more, and more preferably 1% by volume or more and less than 20% by volume. Further, the total amount of the R-rich phase and the R(Fe,Co)₂ phase formed is still more preferably 1.5% by volume or more and less than 15% by volume, and even more preferably 2% by volume or more and less than 10% by volume. In such a range, an area in contact with the main phase grains is secured, and an effect of increasing H_{cJ} is easily obtained. In addition, a decrease in Bᵣ is also suppressed, and desired magnetic properties are easily obtained.

In addition, the anisotropic rare earth sintered magnet of the present invention may contain R oxide, R carbide, R nitride, M carbide, and the like formed by C, N, and O inevitably mixed therein. From the viewpoint of suppressing deterioration of magnetic properties, the volume fraction thereof is preferably equal to or less than 10% by volume, more preferably equal to or less than 5% by volume, and particularly preferably equal to or less than 3% by volume.

It is preferable that the number of phases other than those described above be as small as possible. For example, when an R₂(Fe,Co,M)₁₇ phase and an R₃(Fe,Co,M)₂₉ phase are present in the magnet structure, the amount of each phase formed should be less than 1% by volume from the viewpoints of the influence on the magnetic properties and the suppression of the decrease in the coercive force due to the influence. In addition, from the viewpoint of ensuring a sufficient ratio of the main phase, it is preferable that each of the (Fe,Co)₂M phase, and RM₃, RM₂, R(Fe,Co)M, R(Fe,Co)₂M₂, and the like, in which R is less than 40 at%, is less than 1% by volume. The total amount of these phases is preferably 3% by volume or less. Furthermore, it is preferable that an α-(Fe,Co) phase is not contained in the anisotropic rare earth sintered magnet of the present invention from the viewpoint of preventing significant deterioration in magnetic properties.

Next, a production method will be described. The anisotropic rare earth sintered magnet of the present invention is produced by a powder metallurgy method. First, in order to prepare a raw material alloy, metal raw materials of R, Fe, Co, and M, alloys, ferroalloys, and the like are used, and adjustment is performed so that a finally obtained sintered body has a predetermined composition in consideration of raw material loss and the like during the production process. These raw materials are melted in a high-frequency furnace, an arc furnace or the like to prepare an alloy. A cooling from the molten metal may be performed by a casting method, or may be performed by a strip casting method. In the case of the strip casting method, it is preferable to prepare the alloy so that the average crystal grain size of the main phase or the average grain boundary phase interval becomes 1 µm or more by adjusting the cooling rate. When it is less than 1 µm, the powder after fine pulverization becomes polycrystalline, and the main phase crystal grains are not sufficiently oriented in the step of compacting in a magnetic field, resulting in a decrease in Bᵣ. When α-Fe is precipitated in the alloy, the alloy may be subjected to heat treatment so as to remove α-Fₑ and increase the amount of the ThMn₁₂ type compound phase formed. As the alloy, an alloy having a single composition may be used, or may be adjusted by preparing a plurality of alloys having different compositions and mixing powders thereof in a later step.

The above-described raw material alloys are coarsely pulverized into powder having an average grain size of 0.05 to 3 mm by a means such as mechanical pulverization using a brown mill or the like or hydropulverization. Alternatively, an HDDR method (hydrogen disproportionation desorption recombination method) used as a production method of an Nd-Fe-B base magnet may be applied. Further, the coarse powder is finely pulverized by a ball mill, a jet mill using high-pressure nitrogen, or the like to obtain a powder having an average grain size of 0.5 to 20 µm, more preferably 1 to 10 µm. If necessary, a lubricant or the like may be added before or after the fine pulverization step. Next, using a magnetic field press apparatus, the alloy powder is compacted while the axis of eazy magnetization of the alloy powder is oriented in an applied magnetic field to form a powder compact. The compacting is preferably performed in a vacuum, a nitrogen gas atmosphere, an inert gas atmosphere such as Ar, or the like in order to suppress oxidation of the alloy powder.

The step of sintering the powder compact is performed in a vacuum or inert atmosphere at a temperature of 800°C or higher and 1400°C or lower using a sintering furnace. When the temperature is lower than 800°C, sintering does not proceed sufficiently, so that high sintered density cannot be obtained, and when the temperature exceeds 1400°C, the main phase of the ThMn₁₂ type compound is decomposed and α-Fe is precipitated. The sintering temperature is particularly preferably in the range of 900 to 1300°C. The sintering time is preferably 0.5 to 20 hours, and more preferably 1 to 10 hours. The sintering may be a pattern in which the temperature is raised and then held at a constant temperature, or a two step sintering pattern in which the temperature is raised to a first sintering temperature and then held at a lower second sintering temperature for a predetermined time may be used in order to refine the crystal grains. Further, sintering may be performed a plurality of times, or a spark plasma sintering method or the like may be applied. The post-sintering cooling rate is not particularly limited, but cooling can be performed until least 600°C or lower, preferably 200°C or lower, at a cooling rate of preferably 1°C /min or more and 100°C /min or less, more preferably 5°C /min or more and 50°C /min or less. In order to improve the coercive force, an aging heat treatment may be further performed at 300 to 900°C for 0.5 to 50 hours. H_{cJ} is improved by optimizing the conditions of sintering and aging according to the composition, powder particle size, and the like. Further, the sintered body is cut and ground into a predetermined shape and subjected to magnetization to obtain a sintered magnet.

On the other hand, as a means of producing an anisotropic rare earth sintered magnet having main phase grains in which the Sm/R ratio in the inner portion of the main phase grains is lower than the Sm/R ratios of the R-rich phase and the R(Fe,Co)₂ phase, for example, a dual-alloy method and a grain boundary diffusion method can be exemplified.

When the dual-alloy method is used, metal raw materials of R, Fe, Co, and M, alloys, ferroalloys, and the like are used to prepare two kinds of raw material alloys having different compositions. Three or more kinds of alloys may be used. At this time, it is preferable to combine alloy A mainly composed of the ThMn₁₂ type compound phase and having a relatively low Sm/R ratio with alloy B having a relatively high R composition ratio and a relatively high Sm/R ratio so as to adjust the average composition to a predetermined composition. These alloys are prepared by a casting method or a strip casting method, and pulverized. The step of mixing each alloy powder may be performed in a coarse powder state before fine pulverization, or may be performed after fine pulverization. Further, compacting and sintering are performed to obtain a sintered body. In order to improve the coercive force, aging heat treatment may be performed.

In the sintered magnets produced by the dual-alloy method, a main phase composed of a ThMn₁₂ type compound is formed mainly by the components of the alloy A, and an R-rich phase, an R(Fe,Co)₂ phase, and an outer shell portion of main phase grains are formed mainly by the components of the alloy B. Therefore, the Sm/R atomic ratio of the R-rich phase or the R(Fe,Co)₂ phase formed in the grain boundary portion is higher than the Sm/R atomic ratio in the inner portion of the main phase grain. Further, a part of Sm in the grain boundary phase substitutes R atoms in the surface layer portion of the main phase grain to form a core-shell structure in which the Sm concentration is different between the surface layer portion and the inner portion of the grain, thereby increasing the coercive force.

On the other hand, in the grain boundary diffusion method, first, a sintered body is prepared in the same manner as described above by a single alloy method or a dual-alloy method. At this time, R in the composition of the sintered body may contain Sm or may not contain Sm.

Next, the obtained sintered body is subjected to grain boundary diffusion of Sm. After the sintered body is cut and ground as necessary, a diffusion material selected from compounds such as a metal, an alloy, an oxide, a fluoride, an oxyfluoride, a hydride, and a carbide containing Sm is provided on the surface thereof in the form of powder, a thin film, a thin strip, a foil, or the like. For example, a powder of the above-mentioned material may be mixed with water or an organic solvent to form a slurry, and the slurry may be coated on the sintered body and then dried, or the above-mentioned substance may be provided as a thin film on the surface of the sintered body by means of vapor deposition, sputtering, CVD or the like. The amount to be provided is preferably 10 to 1000 µg/mm², and particularly preferably 20 to 500 µg/mm². Within such a range, an increase in H_{cJ} can be sufficiently obtained, and an increase in production cost due to an increase in the Sm content can be suppressed. Further, by utilizing the property of high vapor pressure of Sm, Sm metal or Sm alloy may be heat-treated together with the sintered body in the same chamber, and brought into contact with the sintered body as Sm vapor.

The sintered body is heat-treated in vacuum or in an inert gas atmosphere in a state where Sm is provided on the surface. The heat treatment temperature is preferably 600°C or higher and a sintering temperature or lower, particularly preferably 700°C or higher and 1100°C or lower. The heat treatment time is preferably 0.5 to 50 hours, and particularly preferably 1 to 20 hours. The cooling rate after the heat treatment is not particularly limited, but is preferably 1 to 20°C/min, and particularly preferably 2 to 10°C /min. In order to improve the coercive force, an aging heat treatment may be further performed at 300 to 900°C for 0.5 to 50 hours.

Sm provided on the sintered body penetrates into the sintered body while increasing the Sm concentration of the R-rich phase or the R(Fe,Co)₂ phase by heat treatment, and the Sm/R ratio of these grain boundary phases is increased. When the Sm concentration in the grain boundary phase becomes high, substitution of R atoms by Sm occurs also in the surface layer portion of the main phase grain in contact with the grain boundary phase, the Sm/R ratio in the surface layer portion of the main phase grain becomes higher than the Sm/R ratio in the inner portion of the main phase grain, and H_{cJ} is increased.

The anisotropic rare earth sintered magnet of the present invention thus produced exhibits a residual magnetic flux density Bᵣ of 5 kG or more and a coercive force H_{cJ} of at least 5 kOe or more, at room temperature. The H_{cJ} at room temperature is more preferably 8 kOe or more. Further, the temperature coefficient β of the coercive force is -0.5%/K or more. Here, β = ΔHcJ/ΔT × 100/H_{cJ} (20°C) (ΔHcJ = H_{cJ} (20°C) - H_{cJ} (140°C), ΔT = 20 - 140 (°C)) is set. The anisotropic rare earth sintered magnet of the present invention has a smaller temperature change in coercive force than that of an Nd-Fe-B sintered magnet, and is suitable for use at high temperatures.

### Examples

Hereinafter, the present invention will be specifically described with reference to Examples and Comparative Examples, but the present invention is not limited to the following Examples.

### [Example 1]

Sm metal, electrolytic iron, Co metal, and V metal were used to control a composition, the composition was melted in an Ar gas atmosphere using a high-frequency induction furnace, and then strip-cast on a water-cooled Cu roll to prepare an alloy thin strip having a thickness of about 0.2 to 0.4 mm. A cross section of this alloy was polished and etched, and then the structure was observed with a laser microscope (LEXT OLS4000 manufactured by Olympus Corporation). The observation was made at a position of about 0.15 mm from the surface where the thin strip was in contact with the cooling roll, and 20 points were observed. For each image, 20 lines parallel to the roll contact surface were drawn at equal intervals, and the number of intersections of these lines with the grain boundary phase portion removed by etching was counted to calculate the average grain boundary phase interval, which was 3.6 pm. After hydrogen storage treatment was performed on the alloy at room temperature, the alloy was subjected to dehydrogenation treatment by heating at 400°C in a vacuum to obtain a coarse powder, and further pulverized by a jet mill in a nitrogen stream to obtain a fine powder having an average gain size of 2.4 pm. Next, the fine powder was filled in a die of a compacting device in an inert gas atmosphere, and was press-formed at a pressure of 0.6 Ton/cm² in a direction perpendicular to a magnetic field while being oriented in the magnetic field of 15 kOe (= 1.19 MA/m) to obtain a powder compact. The obtained powder compact was sintered in an Ar gas atmosphere at 1130°C for 3 hours, cooled to room temperature at a cooling rate of 13°C /min, taken out once, and further subjected to heat treatment in an Ar gas atmosphere at 480°C for 1 hour as an aging treatment to obtain a sintered body sample.

The obtained sintered body sample was analyzed by high-frequency inductively coupled plasma optical emission spectrometry (ICP-OES) using a high-frequency inductively coupled plasma optical emission spectrometer (SPS3520UV-DD manufactured by Hitachi High-Tech Science Corporation), and as a result, the composition was Sm_{10.9}Fe_{bal.}Co_{5.4}V_{14.2}. From the X-ray diffraction measurement of a powder obtained by pulverizing a part of the sample, it was confirmed that the crystal structure of the main phase was ThMn₁₂ type. In addition, the structure of the sintered body was observed and the composition of each phase was analyzed using an EPMA apparatus (JXA 8500F manufactured by JEOL Ltd. ), and it was confirmed that an R-rich phase and an R(Fe,Co)₂ phase were present in an amount of 1% by volume or more in a grain boundary portion. The volume fraction of each phase is calculated as being equal to the area ratio in the backscattered electron image. No R₂(Fe,Co,M)₁₇ phase, R₃(Fe,Co,M)₂₉ phase or α-Fe phase was observed. Since a phase such as an oxide is also present, the total phase ratio is less than 100%. Based on the analysis values of the R(Fe,Co)₂ phase, an alloy having the same composition was prepared by arc melting, subjected to homogenization treatment at 830°C for 10 hours, and then subjected to magnetization-temperature measurement with VSM. The Curie temperature T_{c} was 366°C.

The average crystal grain size of the main phase calculated from the results of etching and observation of the sintered body sample was 8.2 pm. Further, when the magnetic properties were measured with a B-H tracer, the room temperature coercive force H_{cJ} was 10.3 kOe. Furthermore, the temperature coefficient β of H_{cJ} was -0.44%/K. The results are shown in Tables 1 to 3.

### [Comparative Example 1]

Sm metal, electrolytic iron, Co metal, and Ti metal were used to control a composition, the composition was melted in an Ar gas atmosphere using a high-frequency induction furnace, and then strip-cast on a water-cooled Cu roll to prepare an alloy thin strip. The average crystal grain size in the minor axis direction of the alloy obtained from an image observed with a laser microscope was 4.7 pm. In the same manner as in Example 1, pulverization and compacting in a magnetic field were performed, followed by sintering in an Ar gas atmosphere at 1170°C for 3 hours, cooling to room temperature at a cooling rate of 13°C/min, and further subjecting to heat treatment in an Ar gas atmosphere at 480°C for 1 hour to obtain a sintered body sample of Comparative Example 1. The composition value of this sintered body sample analyzed by ICP method was Sm_{10.7}Fe_{bal.}Co_{5.2}Ti_{8.0}. It was also confirmed by X-ray diffraction measurement that the main phase of this sintered body sample was a ThMn₁₂ type crystal. When the formed phase was examined by EPMA, an R(Fe,Co)₂ phase existed, but an R-rich phase was not formed, and a fine (Fe,Co)₂Ti phase was precipitated. Further, the average crystal grain size of the main phase calculated in the same manner as in Example 1 was 8.8 pm. This sintered body sample showed only a low coercive force of 0.1 kOe at room temperature. The results are shown in Tables 1 to 3.

### [Example 2]

Sm metal, electrolytic iron, ferrovanadium, Al metal, and Si were used to control a composition, and the composition was melted in an Ar gas atmosphere by a high-frequency induction furnace to prepare a cast alloy. In order to eliminate the primary α-Fe, the alloy was subjected to heat treatment at 900°C for 50 hours. The structure of the obtained alloy was observed with a laser microscope, and it was confirmed from the observed image that the average crystal grain size of the main phase was 5 pm or more. After hydrogen storage treatment was performed on the alloy, the alloy was subjected to dehydrogenation treatment by heating at 400°C in a vacuum to obtain a coarse powder, and pulverized by a jet mill in a nitrogen stream to obtain a fine powder having an average grain size of 1.8 pm. Further, the fine powder was filled in a die of a compacting device in an inert gas atmosphere and compacted in a magnetic field to obtain a powder compact. The powder compact was sintered in an Ar gas atmosphere at 1140°C for 3 hours, and then cooled to room temperature at a cooling rate of 13°C/min to obtain a sintered body sample.

The composition of the sintered body analyzed by the ICP method was Sm_{9.6}Fe_{bal.}V_{14.4}Al_{0.4}Si_{0.2}. Further, it was confirmed by X-ray diffraction that the crystal structure of the main phase was ThMn₁₂ type. In the grain boundary portion of the sintered body structure, an R-rich phase and an R(Fe,Co)₂ phase were present each in an amount of 1% by volume or more. The H_{cJ} at room temperature measured with a B-H tracer was 8.3 kOe, and the temperature coefficient β of H_{cJ} was -0.46%/K. Further, the average crystal grain size of the main phase calculated in the same manner as in Example 1 was 9.5 µm. Based on the analysis values of the R(Fe,Co)₂ phase, an alloy having the same composition was prepared by arc melting, subjected to homogenization treatment at 850°C for 20 hours, and then subjected to magnetization-temperature measurement with VSM. The Curie temperature T_{c} was 349°C. The results are shown in Tables 1 to 3.

### [Examples 3 to 9]

In the same manner as in Example 2, cast alloys were prepared by high-frequency melting while controlling compositions. In order to eliminate the primary α-Fe, the alloys were subjected to heat treatment at 850 to 1100°C for 10 to 50 hours. The structures of the obtained alloys were observed with a laser microscope, and it was confirmed from the observed images that the average crystal grain size of the main phase was 1 µm or more in all cases. After hydrogen storage treatment was performed on the alloys, the alloys were subjected to dehydrogenation treatment by heating at 400°C in a vacuum to obtain coarse powders, and the coarse powders were pulverized by a jet mill in a nitrogen stream to obtain fine powders having an average grain size of 2 to 4 pm. Further, the fine powder was filled in a die of a compacting device in an inert gas atmosphere and compacted in a magnetic field to obtain a powder compact. The powder compact was sintered in an Ar gas atmosphere, cooled to room temperature, and further subjected to aging heat treatment to obtain a sintered body sample. Table 1 shows the composition of each sample analyzed by the ICP method, the crystal structure of the main phase confirmed by X-ray diffraction, and the average crystal grain size of the main phase of the sintered body. Table 2 shows the sintering treatment conditions, the cooling rate after sintering, the aging treatment conditions, Bᵣ and H_{cJ} measured at room temperature, and the temperature coefficient β of H_{cJ} in each example. In Examples 7 and 8, a two step sintering method was applied in which the temperature was raised to a first sintering temperature, then immediately lowered to a second sintering temperature, and held for a predetermined time. Table 3 shows the composition of each phase analyzed by EPMA and the phase ratio. In each of the samples of Examples 3 to 8, the R-rich phase and the R(Fe,Co)₂ phase were formed in the grain boundary portion, and the samples showed the coercive force of 5 kOe or more at room temperature and the temperature coefficient β of -0.5%/K or more.

### [Comparative Examples 2 to 6]

Sintered body samples of Comparative Examples 2 to 5 were prepared in the same manner as in Example 2 except that the compositions were controlled to those shown in Table 1. The results are shown in Tables 1, 2 and 4. In Comparative Example 2, the total amount of R was less than 7 at%, sufficient sintering could not be performed, and a large amount of α-Fe phase was formed in the sintered body. In Comparative Example 3, the total amount of R exceeded 15 at%, and the volume fraction of the main phase was less than 80%. In Comparative Example 4, the total amount of the M element exceeded 20 at%, the R-rich phase was not observed, and an RFeSi phase of PbClF type crystal was formed. In Comparative Example 5, an RCu₂ phase of KHg₂ type crystal was present at the grain boundary triple junctions, but the total amount of the M element exceeded 20 at%, and the R-rich phase was not observed. In Comparative Example 6, the total amount of M was less than 4 at%, ThMn₁₂ type crystal was not observed in the structure, and a main phase of a Th₂Zn₁₇ type crystal was formed.

### [Comparative Example 7]

Sm metal, electrolytic iron, Ti metal, and V metal were used to control a composition, and the molten raw material was cooled on a Cu roll rotating at a peripheral speed of 20 m/sec to prepare a quenched thin strip raw alloy. The thickness of the thin strip was 10 to 50 µm. The structure of the obtained alloy was observed with a laser microscope, and it was confirmed from the observed image that the average crystal grain size was too fine to be measured, but was at least smaller than 1 µm. After this alloy thin strip was pulverized by a ball mill, a powder having a size of 300 pm or less was selected by a sieve, and hot-pressed in an Ar atmosphere at 750°C. The average crystal grain size of the main phase grains was as fine as about 0.2 to 0.3 µm, and the compositions of the main phase and the grain boundary phase could not be identified by EPMA. In addition, since the axis of easy magnetization of the main phase was not aligned, only low Bᵣ was obtained. The results are shown in Tables 1, 2, and 4.

### [Example 10]

Ce metal, electrolytic iron, Co metal, V metal, pure silicon, and sponge titanium were used to control a composition, the composition was melted in an Ar gas atmosphere using a high-frequency induction furnace, and strip-cast on a water-cooled Cu roll to prepare a quenched thin strip alloy having a composition of Ce 8 at%, Co 1.2 at%, V 12 at%, Si 2.6 at%, Ti 0.8 at%, with the balance being Fe. The average crystal grain size in the minor axis direction of the alloy obtained from an image observed with a laser microscope was 4.5 pm. The alloy was subjected to hydrogen storage treatment at room temperature and then to dehydrogenation treatment by heating at 400°C in a vacuum to obtain a coarse powder (referred to as 10A powder). On the other hand, using Sm metal and electrolytic iron as raw materials, an alloy ingot having a composition of Sm 35 at% and the balance Fe was prepared by using a high-frequency induction furnace, and was made into a coarse powder by mechanical pulverization (10B powder). The 10A powder and the 10B powder were mixed at a weight ratio of 92:8 and then pulverized by a jet mill in a nitrogen stream to prepare a fine powder having an average grain size of 2.4 pm.

This mixed powder was compacted in a magnetic field in the same manner as in Example 1, sintered in an Ar gas atmosphere at 980°C for 3 hours, cooled to room temperature at a cooling rate of 10°C/min, and further subjected to heat treatment in an Ar gas atmosphere at 480°C for 1 hour to obtain a sintered body of Example 10. The composition value of the sintered body sample was Sm_{2.8}Ce_{7.5}Fe_{bal.}Co_{1.5}V_{11.1}Si_{2.4}Ti_{0.8}. It was also confirmed by X-ray diffraction measurement that the main phase of this sintered body was a ThMn₁₂ type crystal. The composition of the main phase measured by EPMA was Ce_{7.8}Fe_{bal.}Co_{1.4}V_{11.7}Si_{2.3}Ti_{0.9} in the central portion of the grain, which does not contain Sm, but was Sm_{5.1}Ce_{2.7}Fe_{bal.}Co_{1.5}V_{11.6}Si_{2.5}Ti_{0.8} in the outer shell portion of the grain, and it was confirmed that the Sm/R ratio in the inner portion of the grain was lower than the Sm/R ratio in the surface portion. The composition analysis values of the R-rich phase and the R(Fe,Co)₂ phase were Sm_{27.7}Ce_{52.4}Fe_{bal.}Co_{1.1}V_{0.1} and Sm_{12.6}Ce_{20.4}Fe_{bal.}Co_{0.6}V_{0.8}Si_{0.1}, respectively, and it was confirmed that the Sm/R ratio in the inner portion of the grains was lower than that of the R-rich phase and the R(Fe,Co)₂ phase. The average crystal grain size of the main phase was 8.6 pm. The coercive force of this sintered body was 10.3 kOe at room temperature, and the temperature coefficient β of the coercive force was -0.44%/K. Based on the analysis value of the R(Fe,Co)₂ phase, an alloy having the same composition was prepared and had a Curie temperature T_{c} of 118°C.

### [Example 11]

Nd metal, electrolytic iron, Co metal, V metal, Al metal, and W metal were used to control a composition, the composition was melted in an Ar gas atmosphere using a high-frequency induction furnace, and then strip-cast on a water-cooled Cu roll to prepare an alloy thin strip having a thickness of about 0.2 to 0.4 mm. The average grain boundary phase interval of this alloy was calculated to be 2.9 pm. After hydrogen storage treatment was performed on the alloy at room temperature, the alloy was subjected to dehydrogenation treatment by heating at 400°C in a vacuum to obtain a coarse powder, and further pulverized by a jet mill in a nitrogen stream to obtain a fine powder having an average grain size of 1.9 µm. Next, the fine powder was press-formed while being oriented in a magnetic field, sintered in a vacuum at 1170°C for 3 hours, cooled to room temperature at a cooling rate of 12°C/min, and taken out to obtain a sintered body.

Then, Sm metal, Co metal and Al metal were introduced into a silica tube having a nozzle hole of 0.5 mm as raw materials, melted at a high frequency in an Ar atmosphere, and then sprayed onto a Cu roll rotating at a peripheral speed of 25 m/sec to prepare a quenched thin strip alloy having a composition of Sm 75 at%, Al 5 at%, with the balance being Co. Further, the quenched thin strip was pulverized by a ball mill for 30 minutes to form a powder having a mass-median grain size of 10.3 µm. The above-described sintered body was dipped into a liquid in which the powder and ethanol were mixed and stirred at a weight ratio of 1:3, pulled up, and then dried with warm air to apply the powder onto the surface of the sintered body. These were subjected to diffusion heat treatment at 880°C for 10 hours in vacuum and further subjected to aging heat treatment in an Ar gas atmosphere at 500°C for 2 hours to obtain a sintered body of Example 11.

As a result of ICP analysis of the sintered body sample of Example 11, the composition was Sm_{1.4}Nd_{9.6}Fe_{bal.}Co_{9.7}V_{13.0}Al_{0.6}W_{0.6}. From the X-ray diffraction measurement of a powder obtained by pulverizing a part of the sample, it was confirmed that the crystal structure of the main phase was ThMn₁₂ type. In addition, the structure of the sintered body was observed and the composition of each phase was analyzed by EPMA, and it was confirmed that an R-rich phase and an R(Fe,Co)₂ phase were present in an amount of 1% by volume or more in a grain boundary portion. No R₂(Fe,Co,M)₁₇ phase, R₃(Fe,Co,M)₂₉ phase or α-Fe phase was observed. Since a phase such as an oxide is also present, the total phase ratio is less than 100%.

The EPMA composition analysis values of the central portion and the outer shell portion of the main phase grains were Nd_{7.7}Fe_{bal.}Co_{9.8}V_{13.8}Al_{0.6}W_{0.6} and Sm_{3.7}Nd_{4.0}Fe_{bal.}Co_{9.9}V_{13.7}Al_{0.6}W_{0.4}, respectively, and it was confirmed that the Sm/R ratio in the inner portion of the grain was lower than the Sm/R ratio in the outer shell portion. The composition analysis values of the R-rich phase and the R(Fe,Co)₂ phase were Sm_{26.7}Nd_{52.1}Fe_{bal}.Co_{17.4}V_{0.4}Al_{0.7} and Sm_{12.3}Nd_{22.3}Fe_{bal.}Co_{4.1}V_{0.1}Al_{0.3}, respectively. While Sm was not detected in the inner portion of the main phase grains, the R-rich phase and the R(Fe,Co)₂ phase present at the grain boundary portion contained Sm and it was confirmed that the Sm/R ratio was high.

Based on the analysis values of the R(Fe,Co)₂ phase, an alloy having the same composition was prepared by arc melting, subjected to homogenization treatment at 800°C for 20 hours, and then subjected to magnetization-temperature measurement with VSM. The Curie temperature T_{c} was 275°C. The average crystal grain size of the main phase calculated from the results of etching and observation of the sintered body of Example 18 was 9.0 pm. Further, when the magnetic properties were measured with a B-H tracer, the coercive force H_{cJ} at room temperature was 8.8 kOe. Furthermore, the temperature coefficient β of H_{cJ} was -0.45%/K.

### [Comparative Example 8]

A sintered body of Comparative Example 9 was prepared in the same manner as the method for preparing the sintered body of Example 11, except that the sintered body was not subjected to powder coating and diffusion heat treatment, but was subjected to aging heat treatment in an Ar gas atmosphere at 500°C for 2 hours.

The composition of the sintered body of Comparative Example 8 was Nd_{9.5}Fe_{bal.}Co_{10.1}V_{12.3}Al_{0.4}W_{0.5} without containing Sm. The composition analysis values of the central portion of the main phase grains and the R(Fe,Co)₂ phase were Nd_{7.9}Fe_{bal.}Co_{10.4}V_{12.8}Al_{0.4}W_{0.5} and Nd_{32.3}Fe_{bal.}CO_{4.5}V_{0.2}Al_{0.1}, respectively, and no R-rich phase was detected. The coercive force H_{cJ} at room temperature of Comparative Example 8 was 0.1 kOe. The results are shown in Tables 5 to 7.

**Table 1**

| | ICP Composition Analysis Value of Sintered Body (at%) | Crystal Structure of Main Phase | Average Crystal Grain Size (µm) |
|---|---|---|---|
| Example 1 | Sm_{10.9} Fe_{bal.} Co_{5.4} V_{14.2} | ThMn₁₂ | 8.2 |
| Comparative Example 1 | Sm_{10.6} Fe_{bal.} Co_{5.1} Ti_{8.0} | ThMn₁₂ | 8.8 |
| Example 2 | Sm_{9.6} Fe_{bal.} V_{14.4} Al_{0.4} Si_{0.2} | ThMn₁₂ | 9.5 |
| Example 3 | Nd_{8.7} Sm_{2.7} Fe_{bal.} Co_{10.1} Si_{12.6} Ga_{0.5} | ThMn₁₂ | 7.2 |
| Example 4 | Sm_{7.3} Ce_{2.9} Fe_{bal.} Co_{1.5} V_{7.9} Ti_{4.1} | ThMn₁₂ | 6.5 |
| Example 5 | Pr_{5.7} Sm_{3.3} Dy_{1.5} Fe_{bal.} Co_{16.0} Cr_{11.4} Al_{1.1} Mo_{2.3} | ThMn₁₂ | 12.1 |
| Example 6 | Sm_{7.7} Gd_{4.0} Fe_{bal.} Co_{25.3} Mn_{3.1} Cu_{0.4} Si_{9.4} W_{0.7} | ThMn₁₂ | 7.7 |
| Example 7 | Nd_{7.5} Sm_{3.9} Zr_{0.6} Fe_{bal.} V_{11.2} Ga_{1.2} Nb_{0.6} Hf_{0.5} | ThMn₁₂ | 8.1 |
| Example 8 | Y_{7.4} Sm_{3.2} Ho_{0.4} Fe_{bal.} Co_{3.9} Cr_{12.6} Ni_{1.0} Ta_{1.5} | ThMn₁₂ | 6.7 |
| Example 9 | Sm_{8.4} Tb_{0.6} Zr_{0.9} Fe_{bal.} Si_{13.5} Al_{1.6} | ThMn₁₂ | 10.1 |
| | | | |
| Comparative Example 2 | Sm_{5.0} Pr_{1.5} Fe_{bal.} V_{11.3} Si_{1.9} | ThMn₁₂ | 5.1 |
| Comparative Example 3 | Nd_{20.8} Sm_{3.4} Fe_{bal.} Co_{20.6} Cr_{9.6} Ga_{2.4} Mo_{0.8} | ThMn₁₂ | 12.1 |
| Comparative Example 4 | Y_{11.4} Sm_{2.4} Fe_{bal.} Si_{19.3} Mn_{2.0} Ta_{3.6} | ThMn₁₂ | 7.9 |
| Comparative Example 5 | Sm_{9.5} Ce_{2.1} Fe_{bal.} Co_{1.8} V_{14.4} Mn_{4.6} Cu_{3.6} | ThMn₁₂ | 8.8 |
| Comparative Example 6 | Pr_{10.1} Sm_{2.8} Fe_{bal.} Co_{3.3} Cr_{1.1} Hf_{1.8} | Th₂Zn₁₇ | 8.3 |
| Comparative Example 7 | Sm_{9.3} Fe_{bal.} V_{4.2} Tis.i | ThMn₁₂ | < 1 µm |

**Table 2**

| | Sintering Condition | Cooling Rate (°C/min) | Aging Condition | Br (kG) | H_{cJ} (kOe) | β (%/K) |
|---|---|---|---|---|---|---|
| Example 1 | 1130°C, 3h | 13 | 480°C, 1h | 9.2 | 10.2 | -0.44 |
| Comparative Example 1 | 1170°C, 3h | 13 | 480°C, 1h | 2.1 | 0.1 | - |
| Example 2 | 1140°C, 3h | 13 | No aging | 8.6 | 8.2 | -0.46 |
| Example 3 | 1150°C, 2h | 20 | 550°C, 2h | 11.5 | 8.5 | -0.48 |
| Example 4 | 1070°C, 3h | 15 | 600°C, 3h | 8.7 | 7.3 | -0.43 |
| Example 5 | 1130°C, 5h | 5 | 480°C, 20h | 7.9 | 2.1 | -0.44 |
| Example 6 | 1160°C, 5h | 25 | 850°C, 6h | 8.6 | 11.5 | -0.49 |
| Example 7 | 1160°C/1060°C, 9h | 10 | 500°C, 3h | 9.3 | 8.9 | -0.45 |
| Example 8 | 1220°C/1140°C, 10h | 8 | 650°C, 5h | 8 | 4.4 | -0.48 |
| Example 9 | 1180°C, 5h | 33 | No aging | 10.8 | 8.7 | -0.42 |
| | | | | | | |
| Comparative Example 2 | 1150°C, 2h | 10 | 700°C, 8h | 0.6 | 0.2 | - |
| Comparative Example 3 | 1160°C, 5h | 30 | No aging | 4.7 | 5.4 | - |
| Comparative Example 4 | 1200°C, 3h | 12 | No aging | 2.5 | 0.6 | - |
| Comparative Example 5 | 1120°C, 3h | 15 | 620°C, 3h | 4.7 | 0.4 | - |
| Comparative Example 6 | 1140°C, 3h | 10 | No aging | 5.4 | 0.2 | - |
| Comparative Example 7 | - | - | - | 4.1 | 6.7 | - |

**Table 3**

| | Constituting Phase | EPMA Composition Analysis Value of Each Phase (at%) | Phase Ratio (% by volume) |
|---|---|---|---|
| Example 1 | R(FeCoM)₁₂ phase | Sm_{7.9} Fe_{bal.} Co_{5.3} V_{14.9} | 91.3 |
| | R-rich phase | Sm_{77.2} Fe_{bal.} Co_{20.8} V_{1.3} | 3 |
| | R(FeCo)₂ phase | Sm_{32.4} Fe_{bal.} Co_{1.0} V_{2.8} | 2.2 |
| Comparative Example 1 | R(FeCoM)₁₂ phase | Sm_{8.0} Fe_{bal.} Co_{5.4} Ti_{7.9} | 89.5 |
| | R(FeCo)₂ phase | Sm_{33.1} Fe_{bal.} Co_{1.0} Ti_{1.5} | 3.7 |
| | (FeCo)₂M phase | Fe_{bal.} Co_{4.3} Ti_{28.0} | 1.9 |
| Example 2 | R(FeCoM)₁₂ phase | Sm_{7.7} Fe_{bal.} V_{14.8} Al_{0.4} Si_{0.2} | 93.8 |
| | R-rich phase | Sm_{59.6} Fe_{bal.} V_{4.8} Al_{0.1} Si_{0.7} | 2.4 |
| | R(FeCo)₂ phase | Sm_{32.5} Fe_{bal.} V_{6.2} Al_{0.6} Si_{0.4} | 1.5 |
| Example 3 | R(FeCoM)₁₂ phase | Nd_{6.0} Sm_{2.1} Fe_{bal.} Co_{10.2} Si_{13.4} Ga_{0.5} | 89.3 |
| | R-rich phase | Nd_{46.7} Sm_{18.7} Fe_{bal.} Co_{24.6} Si_{1.2} Ga_{0.0} | 3.3 |
| | R(FeCo)₂ phase | Nd_{10.8} Sm_{18.0} Fe_{bal.} Co_{1.6} Si_{2.1} Ga_{0.1} | 2.7 |
| Example 4 | R(FeCoM)₁₂ phase | Sm_{5.4} Ce_{2.2} Fe_{bal.} Co_{1.6} V_{8.3} Ti₄.₁ | 91.5 |
| | R-rich phase | Sm_{34.4} Ce_{43.5} Fe_{bal.} V_{0.7} Ti_{0.4} | 1.9 |
| | R(FeCo)₂ phase | Sm_{12.4} Ce_{17.5} Fe_{bal.} Co_{0.3} V_{1.3} Ti_{0.6} | 2.4 |
| | (FeCo)₂M phase | Fe_{bal.} Co_{1.3} Ti_{28.0} | 0.6 |
| Example 5 | R(FeCoM)₁₂ phase | Pr_{3.7} Sm_{2.9} Dy_{1.5} Fe_{bal.} Co_{16.3} Cr_{11.9} Al_{1.1} Mo_{2.4} | 92.7 |
| | R-rich phase | Pr_{41.4} Sm_{18.4} Dy_{1.1} Fe_{bal.} Co_{27.2} Cr_{1.0} Al_{0.1} Mo_{0.2} | 2.3 |
| | R(FeCo)₂ phase | Pr_{8.1} Sm_{18.2} Dy_{1.6} Fe_{bal.} Co_{3.0} Cr_{2.2} Al_{0.2} Mo_{0.4} | 1.7 |
| Example 6 | R(FeCoM)₁₂ phase | Sm_{4.8} Gd_{3.5} Fe_{bal.} Co_{26.6} Mn_{3.3} Cu_{0.3} Si_{10.1} W_{0.7} | 87.7 |
| | R-rich phase | Sm_{37.0} Gd_{21.7} Fe_{bal.} Co_{21.3} Mn_{0.3} Cu_{8.7} Si_{0.9} W_{0.1} | 3.3 |
| | R(FeCo)₂ phase | Sm_{16.9} Gd_{9.6} Fe_{bal.} Co_{10.3} Mn_{1.3} Cu_{0.1} Si_{3.9} W_{0.3} | 4.6 |
| Example 7 | R(FeCoM)₁₂ phase | Nd_{3.8} Sm_{3.4} Zr_{0.6} Fe_{bal.} V_{12.0} Ga_{1.2} Nb_{0.6} Hf_{0.5} | 88.1 |
| | R-rich phase | Nd_{66.0} Sm_{17.0} Fe_{bal.} V_{1.0} Ga_{6.2} Nb_{0.1} Hf_{0.0} | 4 |
| | R(FeCo)₂ phase | Nd_{16.7} Sm_{13.4} Fe_{bal.} V_{2.2} Ga_{0.2} Nb_{0.1} Hf_{0.1} | 3.4 |
| Example 8 | R(FeCoM)₁₂ phase | Y_{5.5} Sm_{2.1} Ho_{0.4} Fe_{bal.} Co_{3.8} Cr_{13.1} Ni_{1.0} Ta_{1.6} | 93.4 |
| | R-rich phase | Y_{0.1} Sm_{69.1} Fe_{bal.} Co_{18.8} Cr_{1.1} Ni_{0.1} Ta_{0.1} | 2.3 |
| | R(FeCo)₂ phase | Y_{0.1} Sm_{29.5} Fe_{bal.} Co_{0.7} Cr_{2.5} Ni_{0.2} Ta_{0.3} | 1.2 |
| Example 9 | R(FeCoM)₁₂ phase | Sm_{6.4} Tb_{0.6} Zr_{0.9} Fe_{bal.} Si_{13.4}Al_{1.6} | 93.3 |
| | R-rich phase | Sm_{61.1} Tb_{1.4} Fe_{bal.} Si_{36.4} Al_{0.3} | 2.8 |
| | R(FeCo)₂ phase | Sm_{28.6} Tb_{1.5} Fe_{bal.} Si_{2.5} Al_{0.3} | 1.3 |

**Table 4**

| | Constituting Phase | EPMA Composition Analysis Value of Each Phase (at%) | Phase Ratio (% by volume) |
|---|---|---|---|
| Comparative Example 2 | R(FeCoM)₁₂ phase | Sm_{5.4} Pr_{1.9} Fe_{bal.} V_{14.4} Si_{2.4} | 73.5 |
| | R-rich phase | - | - |
| | R(FeCo)₂ phase | Sm_{21.1} Pr_{8.7} Fe_{bal.} V_{2.7} Si_{0.4} | 1.9 |
| | α-Fe phase | Fe_{bal.} V_{3.4} Si_{0.6} | 22.8 |
| Comparative Example 3 | R(FeCoM)₁₂ phase | Nd_{9.8} Sm_{0.5} Fe_{bal.} Co_{24.6} Cr_{14.2} Ga_{2.4} Mo_{1.2} | 54.5 |
| | R-rich phase | Nd_{57.0} Sm_{1.1} Fe_{bal.} Co_{24.9} Cr_{1.2} Ga_{4.6} Mo_{0.1} | 23.1 |
| | R(FeCo)₂ phase | Nd_{8.0} Sm_{18.5} Fe_{bal.} Co_{4.6} Cr_{2.7} Ga_{0.4} Mo_{0.2} | 15 |
| Comparative Example 4 | R(FeCoM)₁₂ phase | Y_{5.9} Sm_{0.9} Fe_{bal.} Si_{16.1} Mn_{2.5} Ta_{4.6} | 70.8 |
| | R-rich phase | - | - |
| | R(FeCo)₂ phase | Y_{0.5} Sm_{29.3} Fe_{bal.} Si_{3.0} Mn_{0.5} Ta_{0.9} | 5.6 |
| | CeFeSi phase | Y_{25.2} Sm_{1.9} Fe_{bal.} Si_{37.7} Mn_{0.6} Ta_{1.1} | 20.4 |
| Comparative Example 5 | R(FeCoM)₁₂ phase | Sm_{5.6} Ce_{1.8} Fe_{bal.} Co_{2.0} V_{16.1} Mns.i Cu_{0.1} | 84.2 |
| | R-rich phase | - | - |
| | R(FeCo)₂ phase | Sm_{14.8} Ce_{15.1} Fe_{bal.} Co_{0.4} V_{3.0} Mn_{1.0} Cu_{0.0} | 3.8 |
| | SmCu₂ phase | Sm_{33.7} Fe_{bal.} Co_{0.5} V_{0.2} Cu_{64.3} | 7.3 |
| Comparative Example 6 | R(FeCoM)₁₂ phase | Pr_{5.8} Sm_{1.8} Fe_{bal.} Co_{3.2} Cr_{3.2} Hf_{5.5} | - |
| | R-rich phase | - | - |
| | R(FeCo)₂ phase | Pr_{9.6} Sm_{20.1} Fe_{bal.} Co_{6.0} Cr_{0.6} Hf_{1.0} | 2.4 |
| | Sm₂Fe₁₇ phase | Pr_{8.1} Sm_{2.5} Fe_{bal.} Co_{3.3} Cr_{1.1} Hf_{1.9} | 93.2 |
| Comparative Example 7 | Composition analysis by EPMA is impossible. | | |

**Table 5**

| | ICP Composition Analysis Value of Sintered Body (at%) | Crystal Structure of Main Phase | Average Crystal Grain Size (µm) |
|---|---|---|---|
| Example 10 | Sm_{2.8} Ce_{7.5} Fe_{bal.} Co_{1.5} V_{11.1} Si_{2.4} Ti_{0.8} | ThMn₁₂ | 8.6 |
| Example 11 | Sm_{1.4} Nd_{9.6} Fe_{bal.} Co_{9.7} V_{13.0} Al_{0.6} W_{0.6} | ThMn₁₂ | 9.0 |
| Comparative Example 8 | Nd_{9.5} Fe_{bal.} Co_{10.1} V_{12.3} Al_{0.4} W_{0.5} | ThMn₁₂ | 8.8 |

**Table 6**

| | Sintering Condition and Diffusion Condition | Cooling Rate (°C/min) | Aging Condition | Br (kG) | H_{cJ} (kOe) | β (%/K) |
|---|---|---|---|---|---|---|
| Example 10 | (Sintering) 980°C, 3h | 10 | 480°C, 1h | 9.2 | 10.3 | -0.44 |
| Example 11 | (Sintering) 1170°C, 3h | 12 | No aging | 12.5 | 8.8 | -0.44 |
| | (Diffusion) 880°C, 10h | 5 | 500°C, 2h | | | |
| Comparative Example 8 | (Sintering) 1170°C, 3h | 12 | 500°C, 2h | 2.5 | 0.1 | - |

**Table 7**

| | Constituting Phase | EPMA Composition Analysis Value of Each Phase (at%) | Phase Ratio (% by volume) |
|---|---|---|---|
| Example 10 | R(FeCoM)₁₂ phase | (Central) Ce_{7.8} Fe_{bal.} Co_{1.4} V_{11.7} Si_{2.3} Ti_{0.9} | 92.3 |
| | | (Outer shell) Sm_{5.1} Ce_{2.7} Fe_{bal.} Co_{1.5} V_{11.6} Si_{2.5} Ti_{0.8} | |
| | R-rich phase | Sm_{27.7} Ce_{52.4} Fe_{bal.} Co_{1.1} V_{0.1} | 2.1 |
| | R(FeCo)₂ phase | Sm_{12.6} Ce_{20.4} Fe_{bal.} Co_{0.6} V_{0.8} Si_{0.1} | 3.1 |
| Example 11 | R(FeCoM)₁₂ phase | (Central) Nd_{7.7} Fe_{bal.} Co_{9.8} V_{13.8} Al_{0.6} W_{0.6} | 90.3 |
| | | (Outer shell) Sm_{3.7} Nd_{4.0} Fe_{bal.} Co_{9.9} V_{13.7} Al_{0.6} W_{0.4} | |
| | R-rich phase | Sm_{26.7} Nd_{52.1} Fe_{bal.} Co_{17.4} V_{0.4} Al_{0.7} | 3.4 |
| | R(FeCo)₂ phase | Sm_{12.3} Nd_{22.3} Fe_{bal.} Co_{4.1} V_{0.1} Al_{0.3} | 3.6 |
| Comparative Example 8 | R(FeCoM)₁₂ phase | Nd_{7.9} Fe_{bal.} Co_{10.4} V_{12.8} Al_{0.4} W_{0.5} | 94.5 |
| | R-rich phase | - | - |
| | R(FeCo)₂ phase | Nd_{32.3} Fe_{bal.} Co_{4.5} V_{0.2} Al_{0.1} | 3.4 |

## Claims

1. An anisotropic rare earth sintered magnet represented by the formula (R₁₋ₐZrₐ)ₓ(Fe_{1-b}Co_{b})_{100-x-y}(M¹_{1-c}M²_{c})_{y} (wherein R is at least one element selected from rare earth elements and Sm is essential; M¹ is at least one element selected from the group consisting of V, Cr, Mn, Ni, Cu, Zn, Ga, Al, and Si; M² is at least one element selected from the group consisting of Ti, Nb, Mo, Hf, Ta, and W; x, y, a, b, and c each satisfy 7 ≤ x ≤ 15 at%, 4 ≤ y ≤ 20 at%, 0 ≤ a ≤ 0.2, 0 ≤ b ≤ 0.5, and 0 ≤ c ≤ 0.9), the magnet comprising 80% by volume or more of a main phase composed of a compound of a ThMn₁₂ type crystal, the main phase having an average crystal grain size of 1 pm or more, and containing an R-rich phase and an R(Fe,Co)₂ phase in a grain boundary portion.

2. The anisotropic rare earth sintered magnet according to claim 1, wherein the R-rich phase and the R(Fe,Co)₂ phase are contained in an amount of 1% by volume or more in total.

3. The anisotropic rare earth sintered magnet according to claim 1 or 2, wherein the R-rich phase contains R in an amount of 40 at% or more.

4. The anisotropic rare earth sintered magnet according to any one of claims 1 to 3, wherein the R(Fe,Co)₂ phase is a phase exhibiting ferromagnetism or ferrimagnetism at room temperature or higher.

5. The anisotropic rare earth sintered magnet according to any one of claims 1 to 4, wherein a Sm/R ratio in an inner portion of the main phase grain is lower than Sm/R ratios of the R-rich phase and the R(Fe,Co)₂ phase.

6. The anisotropic rare earth sintered magnet according to any one of claims 1 to 5, wherein a Sm/R ratio in an inner portion of the main phase grain is lower than a Sm/R ratio in an outer shell portion of the main phase grain.

7. The anisotropic rare earth sintered magnet according to claim 5 or 6, wherein Sm is not contained in an inner portion of the main phase grain.

8. The anisotropic rare earth sintered magnet according to any one of claims 1 to 7, wherein the magnet exhibits a coercive force of 5 kOe or more at room temperature, and a temperature coefficient β of the coercive force is -0.5%/K or more.

9. A method for producing the anisotropic rare earth sintered magnet according to any one of claims 1 to 8, comprising: pulverizing an alloy containing a compound phase of a ThMn₁₂ type crystal; compacting the pulverized alloy under application of a magnetic field to form a compact; and then sintering the compact at a temperature of 800°C or higher and 1400°C or lower.

10. The method for producing an anisotropic rare earth sintered magnet according to claim 9, comprising: pulverizing and mixing an alloy containing a compound phase of a ThMn₁₂ type crystal and an alloy having a higher R composition ratio and a higher Sm/R ratio; and compacting the mixture under application of a magnetic field to form a compact.

11. The method for producing an anisotropic rare earth sintered magnet according to claim 9 or 10, comprising: bringing a material containing Sm into contact with a sintered body having a compound phase of a ThMn₁₂ type crystal as a main phase; and subjecting to heat treatment at a temperature of 600°C or higher and a sintering temperature or lower to diffuse Sm into the sintered body.

12. The method for producing an anisotropic rare earth sintered magnet according to claim 11, wherein the material containing Sm to be brought into contact with the sintered body is at least one selected from Sm metal, Sm-containing alloy, Sm-containing compound, and Sm-containing vapor, and a form thereof is at least one selected from powder, thin film, thin strip, foil, and gas.

13. The method for producing an anisotropic rare earth sintered magnet according to any one of claims 9 to 12, comprising subjecting the sintered body to heat treatment at a temperature of 300 to 900°C.
